

Oct. 29, 1940.

B. GASPAR

2,219,305

PHOTOGRAPHIC MULTILAYER MATERIAL FOR COLOR PHOTOGRAPHIC PURPOSES

Filed Dec. 3, 1938

Fig. 1.



Inventor

Beta Gaspar.

F. Gerald Toge

Attorney

## UNITED STATES PATENT OFFICE

2,219,305

PHOTOGRAPHIC MULTILAYER MATERIAL  
FOR COLOR PHOTOGRAPHIC PURPOSES

Béla Gáspár, Hollywood, Calif.

Application December 3, 1938, Serial No. 243,889  
In Great Britain December 9, 1937.

5 Claims. (Cl. 95—2)

The present invention relates to a photographic multilayer material for color photographic purposes. Some or all of the various light-sensitive layers contain, even before the exposure, the dye necessary for the formation of the final image. As is known, such light-sensitive materials after exposure of the light-sensitive layers, are converted into colored pictures by means of local removal of the dyestuff. If two or more layers are arranged upon the same support, it is necessary to sensitise at least two of the layers for differently colored light in order to produce the desired color selection picture in each individual layer with light corresponding to the sensitivity. A suitable sensitisation has been described in my United States Patent Office No. 1,985,344, dated Dec. 25, 1934. In the case of a printing material with a transparent support and with colored layers arranged on one or both sides thereof, as used for the production of color films or transparencies, the first and the rear layer can be printed if desired from each side respectively. In this case these two layers may have the same sensitivity while the colored layer lying between acts optically as a screen. Thus, for example, in my United States Patent 2,183,393, Dec. 12, 1939 describing a three-layer film, an intensively colored yellow emulsion layer lies between two blue-sensitive layers of which the one is colored purple-red and the other blue-green, the yellow dyestuff serving for the composition of the image and acting as a filter during the printing operation.

Now it has been found that it is not possible in all cases to limit the exposure of a blue-sensitive layer or, in the case above referred to, of the two blue-sensitive layers, to these layers. Sometimes the yellow-colored silver halide layer behind the blue-sensitive layer or the middle layer in the above mentioned example is also influenced by the light used for the exposure of the outer layers. The same phenomenon appears not only in the example described of a yellow layer, but also can be observed, if green light falls upon a purple-colored layer, containing a sensitizer which renders it sensitive for green light as, for example, the middle layer of the material shown in Figure 1 of my United States Patent No. 1,985,344, if this layer be rendered sensitive to red by a panchromatic sensitizer which imparts a sensitivity to green light in addition to the sensitivity to red light. This undesired exposure results in a small defect of the prints, hardly visible during projection, but undesirable in view of the modern requirements and disadvantageous in

certain cases as, for example, in the copying of such a picture.

It has been found that the phenomenon described above can be suppressed by increasing the concentration of the dye to such an extent that the layer is more effectively screened against the action of light complementary to the color of the layer. The concentration required for effectively shielding the layer is, however, higher than that required for correct color reproduction. Thus, the problem is not only the increase in dyestuff concentration but further the surplus of the dye must be removed during the process and preferably without an increase of the treatment time.

The subject of the present invention is a material having a sufficiently high concentration of dye for the color separation and allowing a quick processing of the material.

For this purpose the layers are dyed to a color intensity higher than required by the most intensely colored parts of the final image and, therefore, sufficiently high for the color separation. Two dyestuffs of very different resistance against the treating solutions are used for this purpose. The image is formed substantially by one of these dyes alone, the other dyestuff being totally removed from the image.

Accordingly, the invention consists of a light-sensitive multilayer silver halide material, in which at least one light-sensitive layer is formed by an emulsion which in its uncolored state would be sensitive not only to light for which the layer is predominantly sensitised and to which it is intended to be exposed but also to light for which a superimposed light-sensitive layer is sensitive or to be exposed. According to the invention the layer is dyed by a mixture of the dyestuff intended to form the final image in the layer and a second dyestuff of similar color. The dyestuff used for the formation of the dyestuff image is fast to ordinary photographic treating solutions and capable of being bleached out under the influence of the silver image. This dyestuff is used in a concentration which corresponds to the color intensity necessary for a reproduction of the most intensely colored parts of the picture. The auxiliary dyestuff is of practically the same color but of much larger bleaching capacity than the dyestuff for the formation of the image and can be totally removed by treating solutions harmless to the image forming dyestuff. The quantity of the auxiliary dyestuff is chosen in such a manner that its absorption in addition to that of the image forming dyestuff is practically sufficient for preventing any light of complementary color

to enter the layer. This image forming dyestuff may be bleached locally preferably prior to but also during or subsequent to the removal or destruction of the auxiliary dyestuff and the destruction has the effect of lowering the color intensity to that required for a reproduction of the most intensely colored parts of the picture.

*Example 1*

10 As shown in Fig. I of the drawing a silver halide emulsion layer sensitised to green or red light and dyed by a mixture of the dyestuff Xylenewalkgelb (Sandoz, Handbuch der Faerberei, 1926, 2nd ed.) and the auxiliary dyestuff 4,4'-methenyl-bis-[1-(p-sulphophenyl)-3-methyl-pyrazolone-5] is arranged between a blue-sensitive silver halide emulsion dyed magenta by the N-methyl-naphtho-quinolinium salt of the dyestuff Tuchecht-brillantrot 2B, and a blue-sensitive silver halide 15 layer dyed blue-green with Pontamine Sky Blue 5 BX (Schultz Farbstofftabellen, 1931, 7th ed., vol. 1, No. 513). The support can be arranged either adjacent to one of the two outer layers or between the layers. If the yellow layer is red-sensitive and is to be exposed from the side of the purple-red layer, the support is preferably arranged between the blue-green and the yellow layer. Suitable concentrations of the dyestuffs are the following:

| 30                                                                                          | Grams per sq. m.<br>layer surface |
|---------------------------------------------------------------------------------------------|-----------------------------------|
| N-methyl-naphtho-quinolinium salt of the dyestuff Tuchechtbrillantrot 2B                    | 1.2                               |
| 35 Triphenyl-guanidine salt of 4,4'-methenyl-bis-[1-(p-sulphophenyl)-3-methyl-pyrazolone-5] | 1                                 |
| Calcium salt of Xylenewalkgelb G                                                            | 1.4                               |
| Pontamine Sky Blue 5BX                                                                      | 0.6                               |

40 The material may be used for the production of dyestuff images in the manner described in my aforementioned Patent 2,183,393. The dyestuff 4,4'-methenyl-bis-[1-(p-sulphophenyl)-3-methyl-pyrazolone-5] and its preparation is described in my application Ser. No. 240,860 filed Nov. 16, 45 1938. The dyestuff is decolorised by an alkaline developer or by solutions containing sulphite or bisulphite compounds.

*Example 2*

50 In Fig. II I have shown that the support which in this case can be opaque, carries a silver halide layer which is colored blue-green with the N-methyl-naphtho-quinolinium salt of the dyestuff Pontamine Sky Blue 5BX and sensitised with 55 cryptocyanine for infra-red light. This layer contains further a destructible blue-green dyestuff, viz., the dyestuff obtained from 1-(p-sulphophenyl)-3-methyl-pyrazolone-5 and glutamic-dialdehyde-dianilide. Instead of being incorporated within the layer the dyestuff may be applied by the aid of a thin gelatin layer containing the auxiliary dyestuff in a concentration of 0.5 g. per sq. m. the gelatin being poured upon the first layer. A silver halide emulsion layer, 60 sensitised to red light by pinacyanole, and colored magenta with the N-methyl-naphtho-quinolinium salt of Tuchechtbrillantrot 2B, is either coated directly on the blue-green layer or layers or on an intermediary layer of colorless gelatin. 65 The magenta layer, its surface or a separate layer lying above contains a red dyestuff which may be, for example, the diphenyl-guanidine salt of the sulphonnic acid derived from methenyl-bis-oxythionaphthene which may be prepared by adding 70 di-phenyl guanidine, dissolved in water with the

addition of acetic acid, to the dyestuff solution. A yellow colored silver halide emulsion as described in Example 1 is sensitised to green and used in front of the other layers.

75 The quantity of dyestuff depends upon the use of the material. In the case of an image on a transparent support for projection or for transparencies, the dyestuff concentrations may be the same as given in Example 1, whereas in a material for the production of colored images on a 10 paper support the concentration of the image-forming dyestuff is decreased to about  $\frac{1}{2}$  or  $\frac{1}{3}$  of the amounts given in Example 1, whereas the concentration of the auxiliary dyestuff is increased correspondingly.

15 As already described in connection with Example 2 the auxiliary dyestuff having the same or similar color as the image-forming dyestuff may be incorporated in an additional or intermediate layer arranged in front of the light-sensitive layer colored with the image-forming dyestuff. The auxiliary layer may also be light-sensitive and in this case should be sensitised for a spectral range which allows a separate exposure of the intermediate layer as described in my copending 20 application Ser. No. 243,886, filed Dec. 3, 1938. In this case the auxiliary dyestuff may be destroyed, after diffuse illumination of the intermediate layer and developing, by the dyestuff destroying agent which locally destroys the dyestuffs within the image-bearing layers, such as, for instance, 5% hydrobromic acid or an acid thiocarbamide solution.

25 What is claimed is:

30 1. Light-sensitive multilayer material comprising a plurality of silver halide emulsion layers dyed with fast dyes necessary for the formation of a multicolor picture, at least one of which is formed by an emulsion which in its uncolored state would be sensitive not only to the light for which the layer is predominantly sensitized and to which it is to be exposed but also to a differently colored light to be used for the exposure of another of said fast dyed light-sensitive layers situated in front thereof, said other layer being 35 both predominantly sensitive to and at least partially transparent to such differently colored light, the fast dyestuff in the layer first referred to being a dyestuff which absorbs said differently colored light transmitted by the superposed layer and being fast to ordinary photographic treating 40 solutions and being capable of being bleached under the influence of the silver image, the dyestuff further being present in a concentration which is necessary for the reproduction of the 45 most intensely colored parts of the picture, a layer of the multilayer material behind said other layer containing additional dyestuff of substantially the same color as the first-named dyestuff but removable by an agent which does not remove the first-named dyestuff, the amount of fast dyestuff and additional dyestuff together being sufficient to prevent any light of complementary color from entering the said first referred to fast-dyed 50 light-sensitive layer.

55 2. Light-sensitive multilayer material comprising a plurality of silver halide emulsion layers dyed with fast dyes necessary for the formation of a multicolor picture, at least one of which is formed by an emulsion which in its uncolored 60 state would be sensitive not only to the light for which the layer is predominantly sensitized and to which it is to be exposed but also to a differently colored light to be used for the exposure of another of said fast dyed light-sensitive lay- 65

70

75

80

85

90

95

ers situated in front thereof, said other layer being at least partially transparent to such differently colored light, the fast dyestuff in the layer first referred to being a dyestuff which 5 absorbs light rays transmitted by the superposed layer and being fast to ordinary photographic treating solutions and being capable of being bleached under the influence of the silver image, the dyestuff further being present in a concentration which is necessary for the reproduction 10 of the most intensely colored parts of the picture, the layer first referred to containing an additional dyestuff of substantially the same color as the first-named dyestuff but removable by an agent which does not remove the first-named dyestuff, the amount of fast dyestuff and additional dyestuff together being sufficient to prevent any light of complementary color from entering the said first referred to fast-dyed light-sensitive layer.

3. Light-sensitive multilayer material comprising a plurality of silver halide emulsion layers dyed with fast dyes necessary for the formation of a multicolor picture, at least one of which is formed by an emulsion which in its uncolored state would be sensitive not only to the light for which the layer is predominantly sensitized and to which it is to be exposed but also to a differently colored light to be used for the exposure of another of said fast dyed light-sensitive layers situated in front thereof, said other layer being at least partially transparent to such differently colored light, the fast dyestuff in the layer first referred to being a dyestuff which 25 absorbs light rays transmitted by the superposed layer and being fast to ordinary photographic treating solutions and being capable of being bleached under the influence of the silver image, the dyestuff further being present in a concentration which is necessary for the reproduction of the most intensely colored parts of the picture, an intermediate layer between the layer first referred to and the said other layer situated in front thereof containing an additional dyestuff of substantially the same color as the first-named dyestuff but removable by an agent which does not remove the first-named dyestuff, the amount of fast dyestuff and additional dyestuff together being sufficient to prevent any light 30 of complementary color from entering the said first referred to fast-dyed light-sensitive layer.

4. A light-sensitive multilayer material comprising a plurality of silver halide emulsion layers, at least one of which is formed by a dyed emulsion which in its uncolored state would be sensitive not only to the light for which the layer is predominantly sensitized and to which it is to be exposed but also to a differently colored light to be used for the exposure of another light-sensitive layer situated in front thereof, said other layer being at least partially transparent to such differently colored light, the layer first referred to being colored with a dyestuff which absorbs said differently colored light transmitted by said other layer, said dyestuff being fast to ordinary photographic treating solutions and being capable of being bleached under the influence of the silver image, said dyestuff further being present in a concentration which is necessary for the reproduction of the most intensely colored parts of the picture, the layer first referred to containing an additional dyestuff of substantially the same color as the first-named dyestuff but removable by an agent which does not remove the first-named dyestuff, the amount of fast dyestuff and additional dyestuff together being sufficient to prevent any of said differently colored light from entering the said first referred to light-sensitive layer.

BÉLA GÁSPÁR. 55